

## UNITED STATES PATENT OFFICE.

MURRAY C. BEEBE, OF CINCINNATI, OHIO, ASSIGNOR TO THE WADSWORTH WATCH CASE COMPANY, OF DAYTON, KENTUCKY, A CORPORATION OF KENTUCKY.

## MEDALLION ETCHING PROCESS.

No Drawing.

Application filed January 19, 1923. Serial No. 613,753.

To all whom it may concern:

Be it known that I, MURRAY C. BEEBE, a citizen of the United States, residing at Cincinnati, in the county of Hamilton and

5 State of Ohio, have invented certain new and useful Improvements in Medallion Etching Processes, of which the following is a specification.

My invention relates to improvements in medallion etching process and it more especially consists of the features pointed out in the annexed claims.

The purpose of my invention is to provide a variable relief etching process that will enable one to produce medallion effects in high or low relief; that is simple in technique; that is also adaptable for machine or hand rotogravure; and that secures variable relief in lines stipple or other 20 effects with a single etching solution thus eliminating the usual graded etching methods in which varying strengths of mordant are used progressively.

With these and other ends in view, I instance such adaptations as will disclose the broad underlying features of my invention without limiting myself to the specific details of procedure or exact proportion of parts described herein.

30 In practically carrying out my invention I may use any single layer coating which when exposed to a luminous image will become variably permeable to a single etching solution. The original may have very deep 35 shadows, brilliant high-lights and graded middle tones or these tonal values may be accentuated or modified at will, though, what is known as a contrasty subject will, in the main be translated into a variable 40 relief on metal better than so-called "flat" images.

In the well known photogravure process advantage is taken of the fact that a ferric chloride mordant, in a saturated solution 45 will penetrate a gelatin coating, such as carbon tissue, with great difficulty; and a diluted solution will penetrate such a coating more rapidly. In ordinary procedure four ferric chloride solutions ranging from 50 32 to 40 degrees Baumé are used. The basic difference between the above described photogravure process and my method lies in

the fact that I take advantage of a uniform thickness film that is made variably permeable when exposed to a luminous image, 55 instead of producing a variable gelatin relief as is done in the usual photogravure or rotogravure processes. A further difference lies in my use of a single mordant with its attendant simplicity instead of several different etching solutions, each of which requires accurate timing with the risk of completely spoiling the result, if the relation of the different etching stages are not properly maintained. 60 65

In the photogravure processes a grained surface in irregular or geometric pattern is used. The retention of such grain in the shadows is vitally necessary in order that the subsequent wiping off of surplus ink 70 does not pull away the ink from the deep shadows. Similar surfaces may also be produced with my process but, as stated above, without the use of a variable relief or staged etching. 75

In case a matt surface relief is desired, I may use an image that has its tonal gradations broken up into half tone dots, vermicular or irregular grain areas without retaining these characteristics in the final relief 80 etching. As the points of the "grain" are etched away toward the end of the etching period a matt surface is produced. This procedure is specifically adaptable to variable relief productions and obviously not to 85 photogravure-purposes.

As an instance of adaptation the following steps of procedure and relation of ingredients is given. I have found that a furfural acetone resin produces a suitable 90 varnish. This is made by combining 50 grams of acetone, 62 grams of furfural with 100 cc. of a 50% solution of sodium hydrate and heating the mixture in a reflux condenser for about thirty minutes which produces a viscous-like varnish. Of this 12 95 grams is mixed with 3 grams of raw furfural and 5 cc. of alcohol. In turn 20 cc. of this last mixture is combined with about 10 cc. of a 12½% solution of iodoform to constitute a light sensitive coating which is applied to the metal surface on which the variable relief or other form of image is to be produced. The coating may be applied in 100

any desired manner by brushing, whirling etc., etc., producing a so-called wet film onto which the desired image is impressed by means of optical projection for about ten 5 minutes.

The image is developed in benzene and turpentine and is thereafter allowed to stand in turpentine to accentuate the selective permeability of the print corresponding to its 10 more soluble portions. In this connection solubility and permeability are used synonymously in the sense of a coating that is more or less porous and not in the sense of being dissolved away.

15 The etching may be done with a cyanide electrolyte when the image is formed on a gold surface and any other cooperating mordant when other metals are used. In the former case I have found that the permeability or the porosity of the furfural coating cooperates readily with well known gold etching solutions that contain a large amount of water. The image is approximately permeable in proportion to its varying 20 luminosity. The deep shadows of the image or opaque portions of the negative or positive obviously constitute dark areas on the coating which remain in their original state. These areas being most permeable 25 permit the mordant to commence etching the metal beneath the coating before other areas which have been made less permeable by the action of light. In other words the luminous portions of the image correspond to the shallowest parts of the variable relief and 30 the highest relief to the darkest part of the image.

A coating, after exposure, having the 35 variable permeability characteristics above described is also amenable to a selective removal of such portions of the coating that have not been acted upon by the light by the use of any desired solvents or through the aid of mechanical abrasion, for instance, by 40 means of finely powdered glass etc., in the etching bath which is delicately applied. However, in any event the resulting etching will be variable in relief in the same sense as when the coating is retained a uniform 45 thickness. In either case the action of the mordant is slowest where the light action has been the strongest.

The use of iodoform in some measure undoubtedly acts as an accelerating agent to the printing process, but it is used more particularly to give a greater degree of porosity to the portions of the image which have been least exposed to light so as to make such areas more permeable to the etching 55 solution, or more soluble if such areas of the coating are to be variably removed. In any event, I do not limit myself to the use of iodoform or to a furfural resin as any other light sensitive coating which reduces 60 its permeability under the action of light

is considered a practical equivalent, quite in contrast to the effect of ferric chlorid on gelatin as heretofore used in photogravure.

Should it be desired to use my method for rotogravure processes, a separate screen impression can be superimposed on the continuous tone image so as to form ink retaining walls in the deepest shadows corresponding to the greatest depth of a variable relief medallion. As a substitute for the geometrically ruled screen, referred to above, any form of irregular grained texture screen may be used, or the plate itself may be dusted over with powdered resin sufficiently scattered to leave open areas between the 70 powdered particles to form a grain.

Reference has been made hereinbefore to the desirability of having an image intended for medallion etching composed of isolated areas or dots, such for instance as when an 80 original is made with charcoal on grained paper so as to secure a stipple effect. In addition the original may be made by means of the air brush and the negative or positive by using a half tone screen and lastly printing such a half tone on my coating with the image slightly out of focus. This also produces a stipple effect causing the coating to become more permeable because of being thinner at the stipple points which facilitates the beginning of the variable action of the etching solution. I do not limit myself to the use of any accessory steps since the broadest feature of my invention is independent of such details however adaptable 90 they may be in meeting various practical exigencies.

What I claim is:

1. The process of variable relief etching, consisting in covering a metallic surface 105 with a light-sensitive coating, in subjecting the same to a luminous image to produce selectively variable permeable areas in the coating comparable to the lights and shades of the image, in subjecting the image impressed coating to a single mordant, and in selectively controlling the variable rate of action of the mordant by means of the variable image areas.

2. The process of variable relief etching, 110 consisting in covering a metallic surface with a light-sensitive coating, in exposing the same to a luminous image to selectively form areas of low and high permeability corresponding to the lights and shades of the 115 image, and in variably subjecting the coating and its supporting surface to the action of an etching agent.

3. The process of variable relief etching, 120 consisting in covering a metallic surface with a light-sensitive coating, in subjecting the coating to a luminous image so as to selectively produce areas of various permeability in the coating, and in variably subjecting the coating and its supporting surface 125 to the action of an etching agent.

130

face to a single etching solution so as to produce a variable relief on said surface.

4. The process of variable relief etching, consisting in covering a suitable surface 5 with a light-sensitive coating, in exposing the coating to a luminous image to thereby produce areas of variable permeability, and in variably subjecting the coating and surface to an etching solution so as to etch the 10 surface deeply corresponding to the more permeable parts of the image and only slightly or not at all corresponding to the variably luminous parts of the image.

5. The process of variable relief etching, 15 which consists in forming image areas in a suitable coating of low permeability and inter-related areas of high permeability, and in translating such areas into a variable

relief metallic surface by variably subjecting the same to an etching agent whose rate of 20 action is dependent on the variable permeability of the image impressed coating.

6. The process of variable relief etching, which consists in covering a suitable surface 25 with a light-sensitive coating, in subjecting said coating to a luminous image composed of varying sized luminous areas so as to form points of high permeability interspersed among other points of low permeability, and in variably subjecting the coating and its supporting surface to an etching agent adapted to change the surface into a 30 variable relief corresponding to the lights and shades of the image.

In testimony whereof I affix my signature.  
MURRAY C. BEEBE.